

## UNITED STATES PATENT OFFICE

GUSTAV REDDELLEN AND WERNER MÜLLER, OF LEIPZIG, GERMANY, ASSIGNEES TO  
AGFA ANSCO CORPORATION, OF BINGHAMTON, NEW YORK, A CORPORATION OF  
NEW YORK

## PHOTOGRAPHIC DEVELOPER

No Drawing. Application filed July 16, 1930, Serial No. 468,451, and in Germany August 19, 1929.

Our present invention relates to a process of developing photographic materials and new photographic developers.

It is based on the observation that with the exception of the compounds which are twice hydroxyethylated at each nitrogen atom, the N-hydroxyethyl derivatives of 2,4-diamino-1-hydroxybenzene or of N-mono-acyl-2,4-diamino-1-hydroxybenzene or of the nucleal substitution products of these compounds are well suited as photographic developers in so far as they contain no nitro groups.

The compounds in question correspond to the general formula



25  $x, x', y, y'$  meaning hydrogen, acyl, hydroxyethyl, at least one of these substituents being the hydroxyethyl, residue and at least one meaning hydrogen.

30 The said compounds are very stable in solid and in dissolved condition are markedly soluble and have the particular property of developing the latent photographic image in a silver halide emulsion without formation of fog, even in solutions free from potassium bromide.

35 The following examples illustrate suitable compositions for photographic developers in accordance with our invention:

## Example 1

40 6.5 grams of the sulfate of 4-hydroxyethylamino-2-acetamino-1-hydroxybenzene, 45 grams of crystallized sodium sulfite, and 25 grams of potassium carbonate are dissolved in 1000 grams of water.

45 The developer has properties similar to those of the developer made from 4-hydroxyethylamino-1-hydroxybenzene.

## Example 2

50 1 gram of the hydrochloride of 2-hydroxyethylamino-4-acetamino-1-hydroxybenzene, 9 grams of crystallized sodium sulfite, and 5 grams of potassium carbonate are dissolved in 200 grams of water.

The developer is of a similar activity but in a steeper gradation, than that of the developer made in accordance with our U. S. Patent 1,758,762.

## Example 3

55

5 grams of the sulfate of 4-hydroxyethylamino-2-amino-1-hydroxybenzene, 45 grams of crystallized sodium sulfite, and 0.1 gram of potassium bromide are dissolved in 1000 grams of water.

This developer is similar in action to the 60 2,4-diamino-1-hydroxybenzene.

## Example 4

65

1. 35 grams of the sulfate of 2-hydroxyethylamino-4-amino-1-hydroxybenzene, 10 grams of crystallized sodium sulfite, and 0.2 grams of potassium bromide are dissolved in 200 grams of water.

## Example 5

70

1. 5 grams of the sulfate of 4-di-[hydroxyethyl]-amino-2-amino-1-hydroxybenzene, 10 grams of crystallized sodium sulfite, and 0.4 gram of potassium bromide are dissolved in 200 grams of water.

This developer is similar in action to that made from 2,4-diamino-1-hydroxybenzene.

## Example 6

75

1 gram of the sulfate of 2-di-[hydroxyethyl]-amino-4-amino-1-hydroxybenzene and 20 grams of crystallized sodium sulfite are dissolved in 200 grams of water.

The developer is similar in action to a developer containing 4-amino-1-hydroxybenzene in the usual dilution.

## Example 7

85

1. 5 grams of the sulfate of 2-di-[hydroxyethyl]-amino-4-amino-1-hydroxybenzene and 9 grams of crystallized sodium sulfite, and 1 gram of potassium bromide are dissolved in 200 grams of water.

This developer is similar in action to a developer of the usual composition containing 2,4-diamino-1-hydroxybenzene.

90

Our present invention is not limited to the foregoing examples or to the specific details given therein. Thus, for instance, we may use as mentioned above nuclear substitution products of the compounds mentioned in the examples or corresponding to the general formula indicated in the second paragraph of this application. As substituents we enumerate, for instance, alkyl groups or halogen. Other additional ingredients

95

100

known in the photography may be added to the developing baths and we contemplate as included within our invention all such modifications and equivalents.

5. Since nitro derivatives of our new developing agents impart to the photographic layers a strong coloration they are not suited for the purpose set forth.

What we claim is:

10. 1. A photographic developer containing together with other developer ingredients a compound of the general formula:



$x, x', y, y'$  meaning H, acyl, hydroxyethyl at least one of these substituents being hydroxyethyl and at least one meaning hydrogen.

25. 2. A photographic developer containing together with other developer ingredients a compound of the general formula:



$x$  and  $y$  meaning H, acyl, hydroxyethyl.

3. A photographic developer containing together with other developer ingredients a compound of the general formula:



$x$  meaning H, acyl, hydroxyethyl.

4. A photographic developer containing together with other developer ingredients 2-acetylamino-4-hydroxy-ethylamino-1-hydroxybenzene.

50. 5. A photographic developer comprising an alkaline solution containing a compound of the general formula:



$x, x', y, y'$  meaning H, acyl, hydroxyethyl at least one of these substituents being hydroxyethyl and at least one meaning hydrogen.

65. 6. A photographic developer comprising

an alkaline solution containing a compound of the general formula:



$x$  and  $y$  meaning H, acyl, hydroxyethyl.

7. A photographic developer comprising an alkaline solution containing a compound of the general formula:



$x$  meaning H, acyl, hydroxyethyl.

8. A photographic developer comprising an alkaline solution containing 2-acetyl-amino-4-hydroxyethylamino-1-hydroxybenzene.

90. 9. The process of developing photographic materials which comprises treating the same with a solution containing a compound of the general formula:



$x, x', y, y'$  meaning H, acyl, hydroxyethyl at least one of these substituents being hydroxyethyl and at least one meaning hydrogen.

105. 10. The process of developing photographic materials which comprises treating the same with a solution containing a compound of the general formula:



$x$  and  $y$  meaning H, acyl, hydroxyethyl.

11. The process of developing photographic materials which comprises treating the same with a solution containing a compound of the general formula:



$x$  meaning H, acyl, hydroxyethyl.

130

12. The process of developing photographic materials which comprises treating the same with a solution containing 2-acetyl-amino-4-hydroxyethylamino-1-hydroxyben-

5 zene.

13. The process of developing photographic materials which comprises treating the same with an alkaline solution containing sodium sulfite and a compound of the

10 general formula:

15



20  $x, x', y, y'$  meaning H, acyl, hydroxyethyl at least one of these substituents being hydroxyethyl and at least one meaning hydrogen.

14. The process of developing photographic materials which comprises treating

25 the same with an alkaline solution containing sodium sulfite and a compound of the general formula:

30



35  $x$  and  $y$  meaning H, acyl, hydroxyethyl.

15. The process of developing photographic materials which comprises treating the same with an alkaline solution containing sodium sulfite and a compound of the

40 general formula:

45



$x$  meaning H, acyl, hydroxyethyl.

50 16. The process of developing photographic materials which comprises treating the same with an alkaline solution containing sodium sulfite and 2-acetylamino-4-hydroxyethylamino-1-hydroxybenzene.

55 In testimony whereof, we affix our signatures.

GUSTAV REDDELLEN.  
WERNER MÜLLER.